

# UNITED STATES PATENT OFFICE.

ARTHUR HOWARD HIGGINS, OF LONDON, ENGLAND, ASSIGNOR, BY MESNE ASSIGNMENTS, TO MINERALS SEPARATION NORTH AMERICAN CORPORATION.

## CONCENTRATION OF ORES.

1,236,933.

Specification of Letters Patent. Patented Aug. 14, 1917.

No Drawing. Application filed September 23, 1914, Serial No. 863,097. Renewed June 2, 1916. Serial No. 101,383.

*To all whom it may concern:*

Be it known that I, ARTHUR HOWARD HIGGINS, a subject of the King of England, residing at 62 London Wall, London, England, 5 have invented certain new and useful Improvements in the Concentration of Ores, of which the following is a specification.

This invention is for improvements in or relating to the concentration of ores and especially to preferential or selective flotation, that is to say to the separation of different metallic sulfids from one another as well as from gangue when flotation processes are used, and the present invention is in 10 some respects a development of that described in the prior United States Patent to Nutter *et al.*, No. 1,067,485, issued July 15, 1913. For the purpose of defining the 15 nature of this invention, it is desirable first 20 to discuss the factors which obtain in froth flotation processes, and for this purpose attention will be particularly directed to apparatus of the sub-aerator type described in my United States Patent No. 1,155,816, 25 issued October 5, 1915, that is to say, to a flotation apparatus in which the particles in the pulp in a comparatively quiet zone in the upper portion of the flotation vessel are subjected to the action of a continuous 30 stream of innumerable minute gaseous bubbles rising to a froth outlet at the top.

An important factor in froth flotation processes is the tendency of a particle to be wetted by water, and conversely the tendency of a particle to become dry or to become attached to a gaseous bubble. The 35 gangue particles have the greatest tendency to be wetted by water, and have the least tendency to be attached to gaseous bubbles. Further comparing galena and blonde, for 40 example, particles of galena appear to have the least tendency to be wetted with water or the greatest tendency to become attached to gaseous bubbles, while blonde particles appear 45 to have a somewhat smaller tendency to be attached to gaseous bubbles. Pyrites appear to have a still greater tendency than galena to be attached to gaseous bubbles.

In a flotation process, particularly if carried 50 out in an apparatus of the type above referred to, it is found that if a finely crushed ore carrying galena and blonde be subjected to classification so as to obtain products containing particles having sub-

stantially the same rate of fall in water, and if such products are subjected to preferential flotation, the determining factor is the tendency of the attachment to air bubbles. For this reason the galena has the greatest tendency to float.

This invention, therefore, is embodied in a process for the selective separation of the different constituents of an ore by flotation, in which the finely crushed ore is classified so as to yield products containing particles having substantially the same rate of fall in water, whereupon these products are separately treated by a preferential flotation process so as to obtain flotation products relatively high in a certain sulfid on the one hand and residues relatively high in another sulfid on the other hand.

In carrying this invention into effect it is found that the conditions most suitable for preferential or selective flotation are as follows:—

The frothing agent employed should be partly soluble in water, such as eucalyptus amygdalina, and the proportion employed should be very small (about 1 or 2 ounces 80 per ton of ore treated; *i. e.* for 4 tons of water). Additions of frothing agent may be made during the treatment if it is desired to increase the rate at which the froth is produced, care being taken to avoid excess. In 85 a number of previous patents relating to this subject reference has been made to the use of solutes, such as acids, alkalies and soluble salts to assist the selection of the air bubbles. A process embodying this invention may involve the use of these agents, and a simple preliminary test of any particular ore would determine the chemical constitution of the solution to be employed. In most of the experiments which led to the 90 present invention the pulp was alkaline containing about 0.1 to 0.3 per cent. of sodium carbonate in solution. Successful results have also been obtained with other salts, such as sodium bicarbonate and sodium sulfate.

The invention is particularly applicable to finely crushed materials, and the more closely classified the material is, the more exact is the selective flotation. Absolute 105 slime (where the particles have practically no rate of fall in water) forms the last member of the series of classified products.

With classified products the air attachment factor is predominant, so that galena will float in preference to blonde, for example, provided there is no chemical agent present which interferes with the relative "wet-ability" of blonde and galena.

The following example illustrates the application of this invention. The test was made in a small laboratory apparatus of the 10 general type described in the specification of my United States Patent No. 1,155,816, issued October 5, 1915.

The ore was ground wet and put through a conical classifying apparatus and the 15 product which settled more slowly in water was No. 4, of which the original assay was 17.35% Zn, 9.74% Pb. The circuit contained 0.088% of dry sodium carbonate on the water. There was added 3 ozs. of eucalyptus per ton of ore and the mixture was 20 agitated for three minutes, during which the first part of the concentrate was removed. It was then agitated for 5 minutes in which the second part of the concentrate was removed and then agitated for 4 minutes during 25 which the third part of the concentrate was removed. There was then added 3 ozs. more of eucalyptus per ton of ore and the mixture was agitated for 6 minutes, during 30 which the fourth part of the concentrate was removed. The results of these four concentrations were as follows:—

|    | Proportion of original in concentrate. | Assay of concentrate.                 | Recovery.              |
|----|----------------------------------------|---------------------------------------|------------------------|
| 35 | 5.0%                                   | { 7.9% Zn.<br>68.8% Pb.<br>2.6% Ins.  | 2.0% Zn.<br>35.6% Pb.  |
| 40 | 11.3%                                  | { 26.8% Zn.<br>41.4% Pb.<br>1.0% Ins. | 18.0% Zn.<br>48.1% Pb. |
|    | 20.8%                                  | { 46.6% Zn.<br>4.4% Pb.<br>2.4% Ins.  | 55.7% Zn.<br>9.4% Pb.  |
| 45 | 8.2%                                   | { 41.3% Zn.<br>2.2% Pb.<br>9.6% Ins.  | 19.5% Zn.<br>1.8% Pb.  |

It will be seen that the first concentrate is rich in lead while the third and fourth 50 are rich in zinc. The second concentrate is a middlings product which would be re-treated. The tailings contain 54.7% of the original weight, assaying 1.6% Zn and 0.9% Pb.

It is important to note that the results 55 may be seriously interfered with if the proportion of solute or of frothing agent be excessive or insufficient; and from the above directions it will be obvious that a few simple preliminary tests will determine the best conditions.

What I claim as my invention and desire to secure by Letters Patent is:—

1. A process of concentrating ores containing mixed metalliferous minerals which

consists in classifying such an ore so as to obtain a plurality of products one of which products is composed of particles having substantially the same rate of fall in water, and thereafter subjecting such classified product to froth flotation treatment so as to preferentially float one of the metalliferous minerals.

70

2. A process of concentrating ores containing mixed metalliferous minerals which 75 consists in classifying such an ore so as to obtain a plurality of products one of which is composed of particles having substantially the same rate of fall in water, and thereafter subjecting such classified product 80 to froth flotation treatment so as to obtain a flotation product relatively high in a certain metalliferous mineral on the one hand and a residue relatively high in another metalliferous mineral on the other hand, 85 and submitting the residue to further froth flotation treatment for the recovery of the metalliferous mineral contained therein.

90

3. A process of concentrating ores containing mixed metalliferous minerals which 95 consists in classifying such an ore in finely crushed condition so as to obtain a plurality of products each composed of particles having substantially the same rate of fall in water, and thereafter subjecting such classified products separately to froth flotation treatment so as to preferentially float one of the metalliferous minerals.

95

4. A process of concentrating ores containing mixed metalliferous minerals which 100 consists in classifying such an ore in finely crushed condition so as to obtain a plurality of products each composed of particles having substantially the same rate of fall in water, and thereafter subjecting the products separately to froth flotation treatment 105 so as to obtain flotation products relatively high in a certain metalliferous mineral on the one hand and residues relatively high in another metalliferous mineral on the other hand, and submitting the residues to further froth flotation treatment for the recovery 110 of the metalliferous mineral contained therein.

105

5. A process of concentrating ores containing mixed metalliferous minerals which 115 consists in classifying such an ore so as to obtain a plurality of products one of which products is composed of particles having substantially the same rate of fall in water, and thereafter 120 subjecting such classified product to froth flotation treatment with subaeration so as to preferentially float one of the metalliferous minerals.

115

6. A process of concentrating ores containing mixed metalliferous minerals which 125 consists in classifying such an ore so as to obtain a plurality of products one of which is composed of particles having substantially the same rate of fall in water, and thereafter 130

subjecting such classified product to froth flotation treatment with subaeration so as to obtain a flotation product relatively high in a certain metalliferous mineral on the one hand and a residue relatively high in another metalliferous mineral on the other hand, and submitting the residue to further froth flotation treatment for the recovery of the metalliferous mineral contained therein.

10 7. A process of concentrating ores containing mixed metalliferous minerals which consists in classifying such an ore in finely crushed condition so as to obtain a plurality of products each composed of particles having substantially the same rate of fall in water, and thereafter subjecting such classified products separately to froth flotation treatment with subaeration so as to preferentially float one of the metalliferous minerals.

15 8. A process of concentrating ores containing mixed metalliferous minerals which consists in classifying such an ore in finely crushed condition so as to obtain a plurality of products each composed of particles having substantially the same rate of fall in water, and thereafter subjecting the products separately to froth flotation treatment with subaeration so as to obtain flotation products relatively high in a certain metalliferous mineral on the one hand and residues relatively high in another metalliferous mineral on the other hand, and submitting the residues to further froth flotation treatment for the recovery of the metalliferous mineral contained therein.

20 9. A process of concentrating zinc-lead ores which consists in classifying such an ore so as to obtain a plurality of products one of which products is composed of particles having substantially the same rate of fall in water and thereafter subjecting such classified product to froth flotation treatment so as to obtain a flotation product relatively high in lead on the one hand and a residue relatively high in zinc on the other hand.

25 10. A process of concentrating zinc-lead ores which consists in classifying such an ore so as to obtain a plurality of products one of which is composed of particles having substantially the same rate of fall in water, and thereafter subjecting such classified product to froth flotation treatment so as to obtain a flotation product relatively high in lead on the one hand and a residue relatively high in zinc on the other hand, and submitting the residue to further froth flotation treatment for the recovery of the zinc contained therein.

30 11. A process of concentrating zinc-lead ores which consists in classifying such an ore in finely crushed condition so as to obtain a plurality of products each composed of particles having substantially the same

rate of fall in water, and thereafter subjecting such classified products separately to froth flotation treatment so as to obtain a flotation product relatively high in lead on the one hand and a residue relatively high in zinc on the other hand.

35 12. A process of concentrating zinc-lead ores which consists in classifying such an ore in finely crushed condition so as to obtain a plurality of products each composed of particles having substantially the same rate of fall in water, and thereafter subjecting the products separately to froth flotation treatment so as to obtain flotation products relatively high in lead on the one hand and residues relatively high in zinc on the other hand, and submitting the residues to further froth flotation treatment for the recovery of zinc contained therein.

40 13. A process of concentrating zinc-lead ores which consists in classifying such an ore so as to obtain a plurality of products one of which products is composed of particles having substantially the same rate of fall in water and thereafter subjecting such classified product to froth flotation treatment with subaeration so as to obtain a flotation product relatively high in lead on the one hand and a residue relatively high in zinc on the other hand.

45 14. A process of concentrating zinc-lead ores which consists in classifying such an ore so as to obtain a plurality of products one of which is composed of particles having substantially the same rate of fall in water, and thereafter subjecting such classified product to froth flotation treatment with subaeration so as to obtain a flotation product relatively high in lead on the one hand and a residue relatively high in zinc on the other hand, and submitting the residue to further froth flotation treatment for the recovery of the zinc contained therein.

50 15. A process of concentrating zinc-lead ores which consists in classifying such an ore in finely crushed condition so as to obtain a plurality of products each composed of particles having substantially the same rate of fall in water, and thereafter subjecting such classified products separately to froth flotation treatment with subaeration so as to obtain a flotation product relatively high in lead on the one hand and a residue relatively high in zinc on the other hand.

55 16. A process of concentrating zinc-lead ores which consists in classifying such an ore in finely crushed condition so as to obtain a plurality of products each composed of particles having substantially the same rate of fall in water, and thereafter subjecting the products separately to froth flotation treatment with subaeration so as to obtain flotation products relatively high in

4

lead on the one hand and residues relatively high in zinc on the other hand, and submitting the residues to further froth flotation treatment for the recovery of zinc contained therein.

17. A process of concentrating zinc-lead ores which consists in classifying such an ore so as to obtain a plurality of products one of which products is composed of particles having substantially the same rate of fall in water, and thereafter subjecting such classified product to froth flotation treat-

ment with subaeration in the presence of a minute quantity of eucalyptus oil so as to obtain a flotation product relatively high in lead on the one hand and a residue relatively high in zinc on the other hand.

In testimony whereof I have signed my name to this specification in the presence of two subscribing witnesses.

ARTHUR HOWARD HIGGINS.

Witnesses:

WILLIAM JAMES WALTON,  
GEORGE BUTTON.